

# UNITED STATES PATENT OFFICE.

JOSEPH A. MENARD, OF SEATTLE, WASHINGTON.

## ABRASIVE COMPOSITION.

1,381,728.

Specification of Letters Patent. Patented June 14, 1921.

No Drawing.

Application filed April 29, 1920. Serial No. 377,558.

To all whom it may concern:

Be it known that I, JOSEPH A. MENARD, a citizen of the United States, residing at Seattle, in the county of King and State of 5 Washington, have invented certain new and useful Improvements in Abrasive Compositions, of which the following is a specification.

This invention pertains to compositions 10 of abrasive character for grinding or lapping, polishing or finishing metallic bodies and surfaces generally, and has for its primary purpose the grinding, lapping or finishing of journals, bearings, slides, ways, 15 valve seats and plugs, and the like, to produce a fine working fit, to reduce to a minimum the friction between such relatively moving bodies or surfaces, and to automatically produce the necessary clearance or oil- 20 film space between machine parts such as shafts and bearings, rotary valve plugs and their seats, etc. It is designed to reduce materially the extent of the tedious and costly scraping operation now commonly resorted 25 to for finishing the finer grades of machine bearings and surfaces.

The underlying or characteristic feature 30 of the invention resides in the production of a composition which, when first applied to or introduced between surfaces or bodies, one or both of which it is desired to bring to a high degree of finish, shall, upon relative movement of such bodies, have a grinding or abrading action or effect, but which, 35 under continued rubbing or working of the opposed surfaces, shall lose its abrading qualities and become a measurably efficient lubricant.

It is desirable that the composition be of 40 stable character so that it may be kept in stock or on hand, be shipped long distances or subjected to varying climatic conditions, without undergoing change, yet be ready, or capable of being made ready at short 45 notice, for application and use. To this end

I first form a base, comprising the dry elements or ingredients of the composition, which are combined and thoroughly commingled, and at the time of or just before 50 application and use of the composition, I add to this base a suitable liquid or semi-liquid lubricant, preferably a lubricating oil of good quality, an appropriate grease, or water. The addition of the liquid element or vehicle should not, however, be

made until near the time of use, because the abrading properties of the composition would in such case be reduced or impaired, and the attainment of the desired result rendered uncertain or improbable. 60

As the composition is to be used for the finishing of various metals and alloys which differ widely in character, and of parts used under differing working conditions or in different relations, the composition will 65 advisably be made to vary more or less as to the ingredients used, as to the relative proportions thereof, and as to the relative fineness of the abrasive ingredient; but there are certain ingredients that are deemed essential, 70 and certain limits within which the proportions of these should be kept. These variations and limits will be pointed out as the description proceeds.

For the base the following ingredients 75 are deemed essential and will, without addition other than the liquid element, give good results, to wit: potassium, carbonate or sulfate of lead, sodium, and an abrasive, which latter may be any one or more of various 80 substances of the calcium group, as marble, limestone, onyx, etc.; or of the silicon group, as porphyry, trachyte, quartz, flint, sandstone, or the like; or silicates, natural or artificial, such as fluorspar, feldspar, 85 fluorid, sand or glass. Combinations of materials from different groups may be used.

Such abrasive substance should, before inclusion in the base, be reduced by crushing, grinding, trituration, or other usual method, 90 to a granular or pulverulent condition, coarser or finer according to the character of the metal or alloy and the place and manner of use, of the part or body to be treated. In practice I have used the abrasive material 95 of such dimensions as will pass through screens varying from 40 to 200 mesh to the square inch, and this range I deem desirable to cover the various applications and uses of the composition. 100

Carborundum and emery are unsuitable abrasives for use in the composition, as they do not break down or work out in use, but continue to cut or abrade so long as present, and hence are liable to injure instead of 105 properly finishing the metal surfaces if any portion of such abrasive remain in contact with the bearing or wearing surface.

In addition to the ingredients above named I find it at times advantageous to include in 110

the base mixture, carbon in pulverulent form, as for instance, lamp black, graphite, or iron oxid, or any one or more of these.

The lead, preferably in the form of carbonate, though lead sulfate may be employed, the sodium, potassium and oil, grease or water, when subjected to rubbing between the surfaces treated, produce a soapy mixture which serves as a vehicle for the abrasive material, and also acts to break down the latter as the work progresses.

The lamp black, when used, serves to some extent as a binder, and also to color the composition so that it contrasts strongly with the metallic body or surface under treatment, and makes more evident to the eye the effect and progress of the work or treatment.

The office of the sodium is to assist in producing the soapy mixture, and in breaking down or neutralizing the cutting properties of the abrasive element or ingredient under the continued rubbing action.

Iron oxid, of which but a very small quantity is used, if any, tends to give a smoothness to and to improve the action of, the composition. The reason for or the theory of its action has not been clearly ascertained, but its stated effect has been noted.

The preferred base or dry composition consists of the following ingredients in the proportions, by weight, stated: potash, from  $\frac{1}{4}$  of 1% to 3% of the total dry mixture; lead carbonate or lead sulfate, from 5% to 30%; sodium, from  $\frac{1}{4}$  of 1% to  $2\frac{1}{2}$ %; abrasive material of the character indicated, from 30% to 92%. If lamp black be employed it should be in the proportion of from 8% to 12% of the total dry mixture, and if iron oxid be added, it should constitute from  $\frac{1}{4}$  of 1% to  $1\frac{1}{2}$ % of such dry mixture.

These as above indicated, constitute the dry base to which is added, preparatory to application and use, a liquid or semi-liquid lubricant, or water, which may widely vary in amount, say from 25% to 500% in bulk, additional or as related to the dry base. In other words, such lubricant should be equal in bulk to from one-quarter to five times the bulk of the dry ingredients. Such liquid ingredient will preferably be a lubricating oil of good quality, lighter or heavier and of greater or less viscosity according to the character of the metal or alloy treated, the mass and weight of the parts, and similar considerations, such as would ordinarily determine the selection of a lubricating oil or grease in the particular situation. Lard oil is preferred, but any medium bodied engine oil will answer well. Water likewise gives quite satisfactory results in the treatment of some metals and alloys.

As above pointed out, the lamp black and iron oxid may, either or both, be used or omitted at will. The composition is deemed

better with than without them, but they are not nor is either of them, essential. They are to be regarded rather as refinements than as necessary ingredients. The same is true as to graphite.

The choice of abrasive material is dependent in a measure upon the character of the metal or alloy to be treated. Thus for Babbitt metal, as also for brass or bronze bearings, an abrasive in the calcium or the silicate group is deemed advisable, silicates being preferred and crushed or pulverized glass serving quite well. For brass valve seats or plugs the abrasive may be of the silicon group, preferably trachyte.

The composition is also found highly efficient for removing rust, as for instance from the barrels of guns, both large and small, pistons, cylinders, and other moving parts of machinery, the abrasive in such case being preferably of the silicate group. It is likewise found admirably suited to the finishing of engine pistons and cylinders while on the block, particularly high speed engines in which the crank-case forms an oil receptacle. As placed upon the block the cylinders and pistons of engines, pumps, and like machines, have relatively rough or "raw" surfaces which in the testing and working down to commercial shape are very liable to become scored, and to entail a quite considerable percentage of loss. By introducing the dry composition into the oil in the crank case of such high speed engines, or with oil, grease, or water, into the cylinders and bearings of engines, pumps, and similar structures, it is taken up by the liquid or semi-liquid element and distributed over the moving surfaces, where under the continued movement and rubbing of the opposed parts, it polishes the surfaces to a high finish and produces the necessary glaze which for actual use should be given to the moving surfaces. In this way the work is automatically or mechanically performed, and with a degree of accuracy difficult or impossible of attainment by any other known means.

As above explained, the effect of the continued rubbing of the composition is to produce a soapy mixture. This, owing to its peculiar character and properties, gradually and in a measure breaks down the abrasive particles, and ultimately coats any which remain between the opposing surfaces so that they lose their cutting power or capacity. As a consequence, the composition may be permitted to remain between the surfaces to which it is applied where, owing to the change which takes place through the continued rubbing, it is converted into and serves as a lubricant, any particles of the abrading material which may remain between said surfaces being rendered inert or incapable of cutting, and being ultimately

carried off by the flooding action of the oil or other lubricant from time to time supplied to the wearing surfaces in the regular use of the machine or device. The composition may, however, be removed when the grinding or finishing action has been carried to the desired point, and such will be a common procedure though not necessarily a universal one. Gasolene, kerosene, or any similar agent may be employed for such removal.

10 The sodium may be used in the form of carbonate, bicarbonate, borate, bi-borate, hydrate, or other.

15 The potassium is best employed in the form of an oxid, a carbonate, or a sulfate.

Having thus described my invention what I claim is:—

1. A composition of matter comprising 20 in substantially the proportions stated, potassium, lead, sodium, an abrasive, and a suitable vehicle, such composition possessing initially, cutting or abrading properties, but convertible through a rubbing action be-

tween opposed parts movable relatively one 25 to the other, into a lubricating mixture.

2. A dry base for an abrading composition, comprising in substantially the proportions and forms stated, potash, lead, sodium, and an abrasive substance in finely com- 30 minuted form.

3. A dry base for abrading compositions, comprising in substantially the proportions and forms stated, potassium, lead, sodium, lamp black, graphite and iron oxid, and an 35 abrasive substance in finely divided form, said ingredients being intimately commingled.

4. An abrading composition comprising 40 in substantially the proportions and forms stated, potash, a lead compound, sodium, an abrasive material in finely comminuted form, and a lubricant serving as a vehicle for the other ingredients.

In testimony whereof I have signed my 45 name to this specification.

JOSEPH A. MENARD.